

O. Jacobi.  
Making White Lead.

No 94,214.

Patented Aug. 31, 1869.



Witnesses

Hermann Spoerle  
John Bentley

Inventor  
Otto Jacobi

# United States Patent Office.

OTTO JACOBI, OF PHILADELPHIA, PENNSYLVANIA.

*Letters Patent No. 94,214, dated August 31, 1869.*

## IMPROVEMENT IN THE MANUFACTURE OF CARBONATE OF LEAD, ACETATE OF COPPER, AND ACETATE OF IRON.

The Schedule referred to in these Letters Patent and making part of the same.

*To all whom it may concern:*

Be it known that I, OTTO JACOBI, of the city and county of Philadelphia, State of Pennsylvania, have invented a new and useful Apparatus and Mode of Manufacturing Carbonate of Lead, Acetate of Copper, and Acetate of Oxide of Iron; and I hereby declare that the following is a full, clear, and exact description thereof, reference being had to the annexed drawings, in which—

Figure 1 is a vertical section of the apparatus, through the line *a b*.

Figure 2 is a vertical section of the same, through the line *c d*.

Figure 3 is a horizontal section, through the line *u y z*, fig. 1.

Figure 4, a horizontal section and top view, through the line *v w y z*.

Figure 5 is a vertical section of the air-pipe *h*.

The nature of my invention consists in the construction of an apparatus which will convert metallic lead into carbonate of lead, (white lead,) metallic copper into acetate of copper, (verdigris,) and metallic iron into acetate of oxide of iron, by means of vapors of acetic acid and carbonic acid, produced in the lower part of the apparatus, and treating, afterward, the products of corrosion of the lead by a solution of carbonate of soda or potash.

To enable others skilled in the art to make and use my invention, I will proceed to describe its construction and operation.

I take a tub, *A*, made of hard wood, bound with iron bands, and wider at the bottom than at the top. About six inches above the bottom of the tub there is another or false bottom, *B*, perforated by holes of one-half inch diameter, one inch distant from each other. This bottom *B* is covered with coarse linen cloth, or similar fabric. Under the false bottom *B*, in the tub, there is a free space, *x*, to which the air from the outside has access, by means of the air-holes *o o o o o*, and from which the vinegar, which collects there, can be drawn off, by a larger hole, *d*, close to the lower bottom. Above the false bottom *B*, covered with cloth, I have three layers of charcoal, *e f g*. The first, or lower layer, *e*, consists of pieces of charcoal of about one inch diameter, the second, or middle layer, *f*, of smaller pieces, and the third, or uppermost, *g*, of charcoal-dust. These layers are piled up each about six to eight inches high, when the tub *a* is six to eight feet high.

Through the middle of these layers of charcoal passes a wooden air-pipe, *h*, open at the bottom, and provided with a perforated head, whose construction is shown in fig. 5, and which gives to the air a free

passage from the open space *x*, below the false bottom *B*, through the charcoal-layers *e f g*, to the upper space of the tub *A*.

The charcoal is covered with a piece of thin muslin or gauze, and above it I have provided a T-shaped inverted pipe *C*, with a row of holes, of one-sixteenth of an inch in diameter, on the lower side, and with a pivot, *k*, in the centre, which turns freely in a hole cut in the top of the head *i* of the air-pipe *h*.

Above this T-shaped pipe *C*, there is a second false bottom *D*, made in halves separated by an open space, *l*, and constructed either of boards, perforated by holes of one and one-half inch diameter, or of laths, with open interstices between them, as shown in figs. 3 and 4. On this false bottom are piled up sheets of lead or copper, or scraps of iron, rolled in spiral form, as shown in figs. 1, 2, and 4, or in other suitable manner, so that the vapors from below have free access to every part of them.

The tub *A* is closed by a wooden cover, *r*, perforated by a centre-hole, *m*, through which the upper end and orifice of the T-shaped pipe *C* project, and by four air-holes *n n n n*, which serve to keep up the draught through the whole apparatus.

When I want to put my apparatus in operation, I raise the temperature of the room in which it stands (in winter-time by artificial heat) to 70° Fahrenheit, and keep up this temperature during the process. I then wet the charcoal in the tub with vinegar, of such strength, that it takes thirty-five to forty grains of bicarbonate of soda to saturate one ounce of it. This is done by pouring in the vinegar through the open orifice of the T-shaped pipe *C*, projecting above the cover *r*, and turning the pipe slowly around.

After the charcoal is thoroughly saturated with vinegar in this manner, I take a quantity of well-fermented molasses, malt-mash, sugar-mash, or any other liquid containing alcohol, and capable of generating acetic acid, and distribute it through the T-shaped pipe over the surface of the charcoal by slowly turning the pipe. The liquid, in filtering through the different layers of charcoal, emits, first, carbonic acid, and is then converted, by the action of the oxygen of the air ascending from below through the air-holes in the false bottom *B* and the air-pipe *h*, into acetic acid, which rises in vapors, and enters the space above the second false bottom *D*, corroding the lead, copper, or iron sheets piled up there, and converting them into carbonate of lead, acetate of copper, or acetate of oxide of iron.

The vinegar, which drops down and collects, during the process, in the open space *x*, below the lower false bottom, is from time to time drawn off, through the

hole *d*, and used to wet the charcoal in the manner described, by distributing it through the T-shaped pipe over the surface of the same.

The chemical action of the oxygen of the air, during the process, keeps up the temperature in the tub high enough for the purpose of vinegar-production, without the aid of artificial heat.

After the process has gone on, in the manner described, for three or four days, a small quantity of white vinegar of commerce is used, to wash off the impurities, collected in the interior of the T-shaped pipe, from the molasses, malt, or sugar-mash used.

When this is done, the T-shaped pipe is drawn up so far that the cross-piece nearly reaches the cover *r* of the tub, then a solution of seven parts of crystallized carbonate of soda, to two hundred parts of water, is poured in through the upper orifice, and the same is slowly turned around, to wet the whole quantity of lead contained in the apparatus. (When acetate of copper or iron is manufactured, this part of the process, of course, is left out.)

After nine or ten days the process is finished, and the oxide of lead is taken out and put in a vessel, containing a small quantity of water. There always remains some acetate of lead mixed with the carbonate. To convert this, the water is drawn off, and a boiling solution of bicarbonate of soda or potash, in proportion of one pound of the alkali to one hundred pounds of the oxide, is poured over it. It is then allowed to rest, and washed afterward with pure water.

(This process can also be dispensed with, in the manufacture of acetate of copper or iron. It is sufficient to scratch off the verdigris from the copper with a copper knife; and with iron, even this is not necessary.)

What I claim as my invention, and desire to secure by Letters Patent, is—

1. The apparatus for making carbonate of lead, acetate of copper, and acetate of oxide of iron, consisting of tub *A*, provided with two false perforated bottoms *B* and *D*, air-pipe *h*, T-shaped distributing-pipe *C*, air-holes *o o o o o o* and *n n n n*, and layers of charcoal, *e f g*, or their equivalents, all arranged and operating as specified.

2. The process of making carbonate of lead, acetate of copper, and acetate of oxide of iron by means of said apparatus, substantially as described.

3. The use of a solution of carbonate of soda or potash, inside and outside of said apparatus, for the purpose of completing the conversion of the acetate of lead into carbonate of lead.

4. The mode of producing vapors of acetic acid and bringing them in contact with metallic lead, copper, or iron, substantially and for the purpose as set forth.

OTTO JACOBI.

Witnesses:

HERMANN SPOERKE,  
JOHN BENTLEY.